

# UNITED STATES PATENT OFFICE.

MOSES H. DAY, OF ROXBURY, MASSACHUSETTS.

## PREPARATION, MANUFACTURE, AND TREATING OF YARN, HEMP, AND OTHER MATERIALS EMPLOYED IN THE MANUFACTURE OF CORDAGE.

SPECIFICATION forming part of Letters Patent No. 320,763, dated June 23, 1885.

Application filed May 5, 1885. (No specimens.)

*To all whom it may concern:*

Be it known that I, MOSES H. DAY, a citizen of the United States, residing at Roxbury, in the county of Suffolk and State of Massachusetts, have invented certain new and useful Improvements in the Preparation, Manufacture, and Treating of Yarn, Hemp, and other Materials Employed in the Manufacture of Cordage, Rope, and Cables in their various forms; and I do hereby declare that the following is a full, true, and exact description of the invention, which will enable others skilled in the art to which it appertains to make and use the same.

In the manufacture of cables, rope, and cordage in their different forms it has long been the custom to use fibrous material, hemp and yarns saturated with pine or fir tar, in order to render the rope or cordage water-proof and to preserve the material from decay. It has also been well known that the tarred yarn, so prepared for manufacture, becomes dry and stiff if exposed to the atmosphere, owing to the evaporation of the essential oil of tar, which takes place rapidly. This stiffness in the yarn is more apparent in cold weather, because the tar, thick and partly fluid at ordinary temperatures, then becomes solidified.

It is desirable on many accounts that the quantity of tar used in the rope should be as great as may be, and that the yarn or cordage may be manipulated and worked at any temperature.

I am aware that fibrous matters have been treated with a preservative composed of about equal weight of fir-tar and naphtha, and I do not, therefore, claim this process as part of my invention. This process, among other drawbacks, reduces the weight of tar about one-half.

I am also aware that a compound composed of certain oils, and of tar or pitch deprived of their mucilage and superabundant acid, or of any resinous matter whatever deprived of its mucilage and superabundant acid, has been used; but my compound contemplates the use of tar in its natural state, and the combination with an oil never before used for this purpose, and in a different and much less proportion than any that has been heretofore used, there-

by gaining the maximum of tar with the minimum of any other ingredient.

I am also aware that the compounds previously spoken of were used to preserve cordage in hot climates, and not for the purpose of rendering more easy their manipulation and manufacture in low temperature.

I have also discovered by my experience that the vegetable oils are not and cannot be regarded as equivalents in their action upon tar in the process of the making of rope and cordage. Neither do the vegetable oils act as the equivalents of any of the animal oils.

My invention consists of the use of the non-siccative cotton-seed oil, which does not, like the other oils, become thick or solid at low temperatures, and which mixes more intimately with the tar, and does not separate from it and rise to the surface of the compound. Neither does it absorb oxygen from the air, leaving a gummy, sticky residue, as do linseed and other like oils. Nor does it volatilize as do the essential oils, or oil of turpentine, tar, &c. Nor does it contain undissolved particles of fatty matter, as do the animal or fish oils, which do not produce a like softness in tarred yarn when used in small quantities; nor mix intimately with the tar when used in larger quantities, and which are expressed from the yarn when subjected to the pressure and strain incident to rope-making, and which leave the cordage thus made with a greasy and dull appearance, and without the luster and brightness that is so desirable.

I apply my compound to the yarn, hemp, or other material during the process of manufacture by saturation or manipulation in any of the ways usually adopted in the treatment of such materials with tar in rope-making; or the material may be saturated before it is needed for use, and be kept in that condition till needed.

After careful experiment I have found that the best results can be obtained by the use of about two per cent. of cotton-seed oil and ninety-eight per cent. of the tar, though this proportion may be slightly changed on account of some variation in the state of the tar or the temperature at which the mixture is made or is to be used. Old tar requires more, and too

green tar less of the oil, but I have found that the compound, in substantially the proportions given above, yields the best results.

What I claim as my invention, and desire to 5 secure by Letters Patent, is—

1. As a new article of manufacture used in the preparation, manufacture, and treatment of yarn, hemp, and other materials employed in the manufacture of cordage, rope, and cables in their various forms, the within-described compound, consisting substantially of two per cent. of cotton-seed oil and ninety-eight per cent. of tar, as set forth.

2. The within-described process of treating yarn, hemp, and other materials used in the 15 manufacture of cordage and rope in their various forms, the same consisting in saturating the said material with a compound of, substantially, two per cent. of cotton-seed oil and ninety-eight per cent. of tar, as set forth.

MOSES H. DAY.

Witnesses:

GEORGE H. BRODHEAD,  
JOHN E. A. HUSSEY.